

May 8, 1934.

A. C. SCOTT

1,957,733

BLASTING CARTRIDGE AND CHARGE

Filed Feb. 25, 1931



INVENTOR

Alexander Crickshank Scott  
by his attorneys  
Byrnes, Stibbins & Blenko

## UNITED STATES PATENT OFFICE

1,957,733

## BLASTING CARTRIDGE AND CHARGE

Alexander Cruickshank Scott, Faversham, England, assignor, by mesne assignments, to Heat-  
ers Limited, London, England

Application February 25, 1931, Serial No. 518,296  
In Great Britain March 4, 1930

8 Claims. (Cl. 52—1)

This invention comprises improvements in and relating to blasting cartridges and charges.

It is an object of this invention to provide an improved form of blasting explosive for use, for example, in coal mines which is characterized by a high degree of safety from risk when exploded in a dangerous atmosphere such as that of a "fiery" mine and which at the same time is safe in transport and storage.

10 Blasting cartridges are known which comprise a cylinder containing compressed carbon dioxide and a heating cartridge in the cylinder which consists of a self-burning mixture and means to ignite the same. The use as the self-burning mixture of a mixture of a chlorate or perchlorate and aluminium powder has been suggested, and also many other explosive bodies, some of which are unsafe in storage and others of which are unsatisfactory in combustion when 15 in use.

According to the present invention, a blasting cartridge of the type comprising a cylinder charged with a compressed inert gas, that is to say a non-supporter of combustion such as carbon dioxide, is provided with a heating element, the essential constituents of which are potassium perchlorate ( $KClO_4$ ) or like oxygen-carrying crystalline body, the crystals of which are intermingled and coated with a proportion of a resinous body. Preferably the resinous body employed is a phenol formaldehyde condensation product such, for example, as that which is known in commerce under the registered trademark Bakelite as resin A or the resin sold as 30 "Elo" resin.

One very advantageous use of the heating element of the present invention is in connection with blasting cartridges of the type shown in United States Patent No. 1,805,541, granted 40 to Dent Ferrell and Arthur W. Helmholtz, and for purposes of illustration the present invention is herein shown as applied to a cartridge of this general type.

The following is a description by way of example of a particular form of a blasting cartridge, in which resin is employed as a fuel, constructed in accordance with this invention. In this example the heating element consists of potassium perchlorate ( $KClO_4$ ) 84%, and Elo resin 50 in the solidified state, 16%.

The perchlorate is finely powdered, and the resin is admixed therewith in the syrupy stage apart from any extraneous solvent. This material is pressed into cakes, hardened by heat and 55 then broken into granules. The size of the gran-

ules is preferably such as would pass through a screen having 30 meshes to the lineal inch but will be retained upon a screen having 120 meshes to the lineal inch, but finer powder or unsifted material can be used if desired. The perchlorate powder prior to incorporation with the resin has a very fine grain of the order of that which would pass a screen having 200 meshes to the lineal inch.

This heating mixture is introduced into a 65 tubular container made of kraft paper with pressed steel end-caps which act as electric terminals. There is packed in the cartridge a capsule of a standard electric igniting fuse. The igniting compound is electrically connected to 70 the terminals.

The drawings are views in longitudinal section of a blasting cartridge of the type hereinabove referred to and showing the improved heating mixture of the present invention applied thereto. Referring to the drawings, it will be noted that the present invention is disclosed as embodied in a cartridge comprising a steel casing 10 which may be, for example, 30 inches in length and about 2½ inches in diameter and 80 having a rupturable sealing disc 11 and a directing cap 12 at the discharge end. The rupturable steel sealing disc is of such a strength as to be capable of expulsion into cap 12 under a pressure less than that which would suffice to burst the 85 walls of the steel container itself. Means 13 are provided for establishing an electrical connection for the heating element and for introducing carbon dioxide into the interior 14 of the cartridge. The carbon dioxide is introduced 90 in the form of snow to the amount of 3 pounds. The amount of heating mixture for this quantity of  $CO_2$  is about 4 ounces, and for larger or smaller quantities pro rata. The cartridge construction will not herein be described in detail 95 inasmuch as it is substantially the same as that shown in the United States patent above referred to.

The heat producing unit 15 comprises a tubular container made of kraft paper, in which the 100 heating mixture is carried and is adapted to be inserted in the position shown in the drawings. The tubular container 15 carries an electrical connection 16 at one end which makes contact with a rupturable sealing disc 11 and an electrical 105 connection 17 at the opposite end thereof, in contact with the plate 18 constituting the other terminal for the electrical circuit. A capsule of a standard electric igniting fuse is packed in the heating mixture contained in the unit and is 110

connected by wires to the connections 16 and 17.

For use, the container is inserted into a bore hole and ignited by an electric current passed through the igniting charge in the center of the 5 heating element. The latter, upon ignition, expands its products of combustion into the carbon dioxide surrounding it through the perforated walls of the heating element and this, together with the intense heat of combustion or explosion 10 of the mixture acting upon the CO<sub>2</sub>, raises the pressure within the container to a sufficient degree to blow out the metal disc at the end thereof. The result is an explosion, any flame of which is completely screened from surrounding 15 combustible gases by the carbon dioxide present in the container. The effect of such an explosion is greatly enhanced according to the present invention by the uniformity of combustion of the heating element and the 20 intensity of the heat produced, while at the same time the material of which the heating mixture is composed is capable of storage over lengthy periods without deterioration or risk of self-ignition.

25 The rate of combustion of the heating compound in the above example can be regulated by varying the size of grain and also the rate and heat of combustion of the heating element can be regulated within wide limits by varying the 30 constituents, using in combination various mixtures of chlorates, and perchlorates and the like and this without rendering the charge subject to undesired alterations during storage. This capability of varying the characteristics of the 35 charge is a valuable feature of the invention.

I claim:—

1. A blasting cartridge of the type comprising a cylinder charged with a compressed inert gas, provided with a heating element the essential constituents of which are potassium perchloro-

rate (KClO<sub>4</sub>) and a resinous body intermingled with and coated upon the crystals.

2. A blasting cartridge as claimed in claim 1, wherein the resinous body is a phenol formaldehyde condensation product.

3. A blasting cartridge as claimed in claim 1, wherein the heating element consists of approximately 84% of potassium perchlorate and approximately 16% of phenol formaldehyde resin in the solidified state.

4. A blasting cartridge as claimed in claim 1, wherein the heating element is in the form of granules such as would pass through a screen having 30 meshes to the lineal inch but will be retained upon a screen having 120 meshes to the lineal inch.

5. A blasting cartridge as claimed in claim 1, wherein the potassium perchlorate, prior to incorporation with the resinous body, is in the form of a powder such as would pass a screen having 200 meshes to the lineal inch.

6. A blasting cartridge comprising in combination a cylinder charged with a compressed inert gas and a heating element therein, the essential constituents of which are an oxygen-carrying 100 crystalline body and a resinous body uniformly distributed therethrough.

7. A blasting cartridge comprising in combination a cylinder charged with a compressed inert gas and a heating element therein, the essential 105 constituents of which are an oxygen-carrying crystalline body and a resinous body insoluble under compressed carbon dioxide.

8. A blasting cartridge comprising in combination a cylinder charged with a compressed 110 inert gas and a heating element therein, the essential constituents of which are an oxygen-carrying crystalline body and a phenol formaldehyde condensation product.

ALEXANDER CRUICKSHANK SCOTT. 115

45

120

50

125

55

130

60

135

65

140

70

145

75

150